# EUROPEAN PATENT SPECIFICATION

(11) **EP 1 011 897 B1**
(45) Date of publication and mention of the grant of the patent: **17.09.2003**
(21) Application number: 98901901.3
(22) Date of filing: 02.02.1998
(51) Int. Cl.: B22D 17/00, B21C 23/00

(54) **SEMI-SOLID METAL FORMING PROCESS**
METALLFORMUNGSVERFAHREN MIT HALBFESTEM MATERIAL
PROCEDE POUR FORMER UN METAL SEMI-SOLIDE

(30) Priority: 31.01.1997 CA 2196479; 23.01.1998 CA 2227828
(43) Date of publication of application: 28.06.2000
(73) Proprietor: Amcan Castings Limited, Hamilton, Ontario L8L 7X3 (CA)
(72) Inventor: WOODHOUSE, Gordon, St. Catharines, Ontario L2T 3R6 (CA)
(74) Representative: Kennedy, David Anthony
(86) International application number: CA9800062
(87) International publication number: WO98033610

(56) References cited:
- US-A- 4 415 374
- M. KIUCHI ET AL.: "MASHY-STATE EXTRUSION, ROLLING AND FORGING" June 1994 , THE 3RD INT'L CONF. ON SEMI-SOLID PROCESSING OF ALLOYS AND COMPOSITES XP002066438 see the whole document

## Description

### FIELD OF THE INVENTION

This invention relates generally to semi-solid metal forming and more particularly to the formation and use of magnesium billets in semi-solid metal die casting and semi-solid forging processes.

### BACKGROUND

Metal die casting is a process in which molten metal is caused to flow into a cavity defined by a mold. In conventional metal die casting, molten metal is injected into the cavity. In semi-solid metal die casting processes, a metal billet is pre-heated to a point of softening, to a temperature above the solidus and below the liquidus to produce a partially solid, partially liquid consistency prior to placing the billet or "slug" in a shot sleeve in the casting machine.

Semi-solid metal die casting enables control of the microstructure of the finished part to a degree which produces a stronger part than is possible with conventional molten metal die-casting processes. As compared with conventional metal die-casting processes, semi-solid metal casting produces parts of improved casting quality in that they exhibit lower porosity, parts shrink less upon cooling enabling closer tolerances and physical properties are better. In addition, semi-solid metal casting has a reduced cycle time and the lower temperatures utilized result in decreased die wear. Because of the absence of molten metal there is less pollution and safety hazards are reduced.

In semi-solid metal die casting, a billet is first formed which is treated to form fine grained equiaxed crystals as opposed to a dentritic structure. Subsequent heating, forming and solidification of a formed part using a treated billet avoids the formation of a dentritic structure in the finished part.

To work successfully in semi-solid metal casting, the grain structure of a billet must exhibit the necessary degree of lubricity and viscosity to give good laminar flow in the die cavity. For example an untreated DC cast billet will shear along its dentritic axis rather than flow hence the need for fine grained equiaxed crystals.

Flowability is further affected by grain size and solid/liquid ratio. In addition forming parameters such as die temperatures and gate velocity will affect the casting process. Accordingly, all of the foregoing parameters have to be optimized in order to produce successful parts.

Metal forging is another process in which metal is caused to flow into a cavity defined by a mold. Unlike die casting, metal is not injected as a liquid into the cavity, but rather a solid billet or slug is placed between dies which are subsequently forced together to squeeze the billet or slug into the cavity as the die is closed. In semi-solid metal forging, the metal billet is pre-heated to a partially solid, partially liquid consistency prior to forging. The consistency is similar to that used for semi-solid metal die casting.

As in semi-solid metal die casting, the billet should consist of fine grained equiaxed crystals rather than a dendritic structure to optimise the flow of metal between the dies and to optimise the physical characteristics of the finished parts.

An earlier process for forming a treated billet involves in the use of magnetic stirring during the cooling of the cast billet to break up and avoid the formation of the dendritic structure. Magnetic stirring is however a relatively slow and expensive process.

US Patent Number 4415374 (Young et al) describes an alternate process forming a billet of aluminium for use in a semi-solid metal die casting process. The object of the process is to produce a fine grained metal composition, and comprises the following steps:
1. Melting and casting an ingot;
2. Cooling the ingot to room temperature;
3. Re-heating the ingot above its recrystallization temperature but below its solidus temperature;
4. Producing a directional grain structure within the ingot by hot working the ingot at a temperature between the re-crystallisation temperature and the solidus temperature. In particular, the hot working includes extrusion of the ingot;
5. Cooling the ingot to room temperature. It is also stated that additional thermal strains may be introduced to the hot working material by rapid chilling of the ingot;
6. Cold working the ingot;
7. Reheating the ingot above its solidus temperature; and,
8. Forming and quenching the ingot, for example by shaping the ingot in a press forging operation .

The ingot produced according to the process described in Young may be shaped during the original reheat of the alloy to a temperature above its solidus temperature, i.e. during step 7. Alternatively, the ingot produced may be subsequently heated to a semi-solid die casting temperature and formed into a part in a die casting process.

Even although Young avoids the requirement for magnetic stirring, it is nevertheless a cumbersome process including a large number of process steps. In particular, a further strain introduction beyond the ingot working extrusion step is required to form an ingot suitable for SSM forming. For example, the Young process requires additional cold working of the ingot (step 6 in the above-described process). This is a consequence of the particular type of starting materials used in the Young process, which are described as direct chill class billets which may or may not be produced under a shearing environment.

More recently the process has been proposed in which a cast ingot machines down a billet to approximately one inch (25 mm) in diameter and deformed by subjection to the compressive force. The deformed billet is then heated to a temperature above its re-crystallisation temperature and below its solidus temperature. The billet is then cooled to room temperature for subsequent re-heating and use in a semi-solid metal casting process. This process however involves an expensive and wasteful machining operation and only appears to work with relatively small billet diameters of less than about one inch (approximately 25 mm) diameter.

It is therefore an object of the present invention to provide a process for semi-solid metal die casting which avoids not only magnetic stirring, but also eliminates many of the steps that would be required pursuant to the Young process.

It is a further object of the present invention to provide a semi-solid metal die casting process which avoids the machining, cold working, heating, cooling and re-heating steps associated with other processes.

It is yet a further object of the present invention to provide a process capable of forming billets for use in semi-solid metal die casting processes that may be significantly greater than about one inch (approximately 25mm) in diameter.

### SUMMARY OF THE INVENTION

According to a first aspect of the invention, there is provided a process for producing a billet for use in a semi-solid metal forming process having the following steps:
i) obtaining a direct chill cast billet which was cooled at a rate exceeding 2°C per second during its production;
ii) heating the direct chill cast billet of step i) to a temperature above its recrystallization temperature and below its solidus temperature;
iii) reducing the diameter of the heated billet from step ii) and breaking down its grain structure by extruding it through an extruding die to form an extruded column; and,
iv) cutting the extruded column to form said billet.

According to a second aspect of the invention, there is provided a billet for use in a semi-solid metal forming process, the billet being obtainable by a process according to the first aspect.

According to a third aspect of the invention, there is provided a semi-solid metal forming process having the following steps:
i) obtaining a direct chill cast billet which, during its production, was cooled at a rate exceeding 2°C per second;
ii) heating the direct chill cast billet to a temperature above its recrystallization temperature and below its solidus temperature;
iii) reducing the diameter of the heated billet from step i) and breaking down its grain structure by extruding it through an extruding die to form an extruded column;
iv) cutting the extruded column into billets;
v) heating the billet from step iv) to a forming temperature above its solidus and below its liquidus temperature;
vi) forming a part from the heated billet by (a) placing the heated billet into an injection chamber in a semi-solid die casting machine, injecting the heated billet section into a mold to form a part; and removing the part from the mold; or (b) placing the heated billet between a set of dies in a forging machine, actuating the forging machine to squeeze the billet between the set of dies to form a part, and separating the dies and removing the part.

### DESCRIPTION OF DRAWINGS

Preferred embodiments of the present invention are described below with reference to the accompanying drawings in which:
Figure 1A is a schematic representation of the process of the present invention;
Figure 1B is a schematic representation of an alternate embodiment process according to the present invention;
Figures 2 through 30 are photomicrographs of billets cut from extruded cast billets and are individually described in Example 1 below;
Figure 31 illustrates sample locations in a test plate which were tested in Example 3;
Figure 32 illustrates the locations at which photomicrographs were taken in Example 3 below; and
Figures 33 through 36 are photomicrographs individually described in Example 3 below.

### DESCRIPTION OF PREFERRED EMBODIMENTS

Referring to Figure 1, molten metal 10 is poured from a ladle into a mold 12 and allowed to solidify into a cast billet 14. The cast billet 14 is heated, for example by inductive heating coil 16 to a temperature above its recrystallization temperature and below its solidus temperature.

The heated cast billet 14 is then extruded through an extruding die 18 to form an extruded column 20. The extruded column 20 is cut to a suitable length billet 22 for use in a semi-solid metal die casting process.

The billet 22 is heated to a forming temperature corresponding to a semi-solid state, for example by induction coils 24, and transferred to a die casting apparatus 26. The heated billet 22 is squeezed by the die casting apparatus into a cavity 28 between mold parts 30 and 32 to form a part 34 conforming in shape to that of the cavity 28.

Alternatively, the heated billet 22 may be transferred to a forging apparatus 40 where it is squeezed into a cavity defined between a movable die 42 and a fixed die 44.

The present invention is further illustrated by the examples set out below.

### EXAMPLE 1

The microstructure of two AZ61 alloy, 3 in. diameter by 7 in. length extruded billets in the as extruded and solution heat treated condition were examined.

The billets were produced initially as an 8 1/2 in. direct chill cast billet. The billets were cooled at a high chill rate utilizing copper molds and a water spray to provide a chill rate of at least 2°C per second at the billet centre. The billets were cut into 2 ft. long sections and the diameter machined down to 8 in. to remove imperfections to the outside edge.

Grain sizing of the 8 inch billet perpendicular to the extrusion axis was 38 microns at the outside, 48 microns at the half radius and 48 microns at the center. As expected, the grain size in the longitudinal or extrusion direction was somewhat larger being approximately 51 microns at the outside, 64 microns at the half radius and 74 microns at the center.

The billets were then heated in 4-6 minute intervals in three induction furnaces. The furnaces heated the billets to 100°C, 200°C, 300°C (total heating time approximately 15 minutes.) The billet was then placed in the extrusion chamber, which was at 380°C and the billet was extruded at between 330°C and 350°C, in one stage down to a 3 in. diameter extrusion billet. The first 14 ft. of extrusion and the last few feet were discarded. The remainder of the extrusion was cut into 7 in. sections or "slugs".

### PROCEDURE

Two of the sections of the extrusion billet referred to as billet 1 and billet 2, in AZ61 alloy were examined in the "as extruded" condition by sectioning a 0.5 in. section off the end of each billet, (billets were randomly selected.) A micro was taken perpendicular to the axis of the billet from the centre and from the outside edge. The micros were polished and etched using 2% nitol etchant. The micros were examined at various magnifications to observe grain structure. A photomicrograph was taken at each magnification and the grain size estimated.

The two extrusion billet sections were then given the following solution heat treatment to recrystallize the grain structure;

| SOLUTION HEAT TREATMENT | |
|---|---|
| Ramp 150°C - 338°C | 3.0 hrs |
| Hold 338°C | 0.1 hrs |
| Ramp 338°C - 413°C | 1.5 hrs |
| Hold 413°C | 0.5 hrs |
| Ramp 413°C - 426°C | 0.5 hrs |
| Hold 426°C | 12.0 hrs |
| Air Cool | |
| (Furnace atmosphere 10% CO₂ to avoid ignition.; | |

The same procedure was followed in billet sectioning polishing and etching as previously described with the "as extruded" billet sections.

From the same samples micros were made at the centre of each billet parallel to the extrusion axis. These micros were taken from the as extruded and the solution heat treated billets. Photo micrographs were made at from 100 x to 400 x magnification of these samples.

The purpose for solution heat treating the extrusion billets and analyzing the samples was to determine the effect on grain size and shape resulting from heating and extruding the DC cast billet. The solution heat treating was not carried out under the optimum circumstances as equipment availability necessitated the use of convection heating rather than induction heating. Preferably the heating cycle should not exceed 20 minutes and accordingly multi-state induction heating would be preferable over convection heating. Nevertheless the results were quite favourable as set out below.

### RESULTS

The photomicrographs which are set out in Figures 2 through 30 below were taken are as follows:
Figure 2 is a photomicrograph of the outside edge of billet 1, as extruded, at 200 x magnification.
Figure 3 is a photomicrograph of the outside edge of billet 1, as extruded at 400 x magnification;
Figure 4 is a photomicrograph of the centre of billet 1, as extruded under 100 x magnification;
Figure 5 is a photomicrograph of the centre of billet 1, as extruded under 200 x magnification;
Figure 6 is a photomicrograph of the outside edge of billet 2, as extruded, at 200 x magnification;
Figure 7 is a photomicrograph of the outside edge of billet 2, as extruded, at 400 x magnification;
Figure 8 is a photomicrograph of the centre of billet 1, as extruded, at 400 x magnification;
Figure 9 is a photomicrograph of the centre of billet 2, as extruded, at 200 x magnification;
Figure 10 is a photomicrograph of the centre of billet 2, as extruded, at 400 x magnification;
Figure 11 is a photomicrograph of the outside edge of billet 1, extruded and solution heat treated, at 50 x magnification;
Figure 12 is a photomicrograph of the outside edge of billet 1, extruded and solution heat treated, at 100 x magnification;
Figure 13 is a photomicrograph of the outside edge of billet 1, extruded and solution heat treated, at 200 x magnification;
Figure 14 is a photomicrograph of the centre of billet 1, extruded and solution heat treated at 50 x magnification;
Figure 15 is a photomicrograph of the centre of billet 1, extruded and solution heat treated at 100 x magnification;
Figure 16 is a photomicrograph of the centre of billet 1, extruded and solution heat treated, at 200 x magnification;
Figure 17 is a photomicrograph of the outside edge of billet 2, extruded and solution heat treated, at 50 x magnification;
Figure 18 is a photomicrograph of the outside edge of billet 2, extruded and solution heat treated, at 100 x magnification;
Figure 19 is a photomicrograph of the outside edge of billet 2, extruded and solution heat treated, at 200 x magnification;
Figure 20 is a photomicrograph of the centre of billet 2, extruded and solution heat treated, at 50 x magnification;
Figure 21 is a photomicrograph of the centre of billet 2, extruded and solution heat treated, at 100 x magnification;
Figure 22 is a photomicrograph of the centre of billet 2, extruded and solution heat treated, at 200 x magnification;
Figure 23 is a photomicrograph of the centre of billet 1, as extruded, parallel to the extrusion axis, at 100 x magnification;
Figure 24 is a photomicrograph of the centre of billet 1, as extruded, parallel to the extrusion axis, at 200 x magnification;
Figure 25 is a photomicrograph of the centre of billet 2, as extruded, parallel to the extrusion axis, at 100 x magnification;
Figure 26 is a photomicrograph of the centre of billet 2, as extruded, parallel to the extrusion axis, at 200 x magnification;
Figure 27 is a photomicrograph of the centre of billet 1 parallel to the extrusion axis, after solution heat treatment, at 100 x magnification;
Figure 28 is a photomicrograph of the centre of billet 1 parallel to the extrusion axis, after solution heat treatment, at 200 x magnification;
Figure 29 is a photomicrograph of the centre of billet 2 parallel to the extrusion axis, after solution heat treatment, at 100 x magnification;
Figure 30 is a photomicrograph of the centre of billet 2 parallel to the extrusion axis, after solution heat treatment, at 200 x magnification;

| Grain Size Determination | |
|---|---|
| As Extruded Billets | |
| Billet 1 Outside Edge | 10.2 microns |
| Billet 1 Centre | 7.6 microns |
| Billet 2 Outside Edge | 7.6 microns |
| Billet 2 Centre | 7.6 microns |
| (Structure is quite broken up with very large and very small grains.) | |

| Solution Heat Treated Billets | |
|---|---|
| Billet 1 Outside Edge | 25.3 microns |
| Billet 1 Centre | 22.5 microns |
| Billet 2 Outside Edge | 22.5 microns |
| Billet 2 Centre | 20.3 microns |
| (Well defined solution heat treated grain structure) | |

### DISCUSSION

The microstructure observed consists of magnesium primary magnesium and aluminum solid solution crystals and eutectic consisting of two phases, secondary magnesium solid solution crystals and Mg₁₇Al₁₂ intermetallic compound. The structure was quite broken up in the "as cast" specimens and grain size measurement is only approximate.

Recrystallized grain structure in the solution heat treated specimens was more accurate and well defined in the microstructure.

The micros taken in the direction of the extrusion axis of the "as extruded" specimens showed long stringers in the microstructure. The corresponding micros taken from the heat treated specimens showed a more evenly distributed recrystallized structure.

The amount of breakdown that the grain structure of the as-cast billet will undergo is likely a function of the amount of reduction. In the present case 7 to 1 reduction was used. Some sources suggest that the optimum degree of reduction should be on the order of from 10:1 to 17:1. In practice however the degree of reduction required may be less if the starting alloy is relatively fine grained.

### EXAMPLE 2

### OVERVIEW

3 in. diameter x 180 mm long slugs of magnesium alloy AZ61 were tested.

10 of the slugs had been solution heat treated.

SSM casting tests were made using a Buhler SCN66 machine. It was not possible at the time of the trials to store the injection curves due to software issues.

As a test piece, a welding test plate die was chosen, heated by oil to approximately 220°C.

In general, the material was SSM-castable, but different than other magnesium alloys. The thickwall part (10mm thick) was perhaps not ideal for magnesium casting.

### SSM HEATING

Slug heating was performed in a single coil induction heater and optimized such that the slugs were removed from the coil just prior to the onset of burning which corresponded to a softness which allowed dissection with a knife. Total heating time was approximately 230 seconds. Very little metal run-off was obtained during the heating process.

A single stage induction heater was utilized for the test as multi-stage induction heating was not available at the test facility. It is expected that better heating would have been obtained with multi-stage induction heating. Ideally at the end of the heating cycle the billet should have a uniform temperature throughout with a well controlled solid to liquid ratio.

### SSM CASTING

The first parts were cast using a plunger velocity of 0.3 to 0.8 meters per second. These conditions barely filled the die and visual laps were apparent at the end of the part.

With a velocity increase to 1.8m/s (onset of flashing), the parts filled better but lapping was still apparent. The best results were obtained using a plunger velocity of 1.2 m/s.

The heat treated slugs appeared lighter in color after heating and had less tendency to burn. The SSM parts produced from these slugs also appeared lighter in color.

Even at plunge velocities as low as 0.05 m/s and up to above 0.5 m/s, it was not possible to achieve a smooth metal front. In all cases the alloy flowed as individual "glaciers".

Two plates (numbers 34 and 35) which were formed at a plunger velocity of 1.8 m/s were subjected to metallurgical evaluation (see Example 3).

As can be seen, the only parameter varied in making the test plates was the gate or plunger velocity. Accordingly none of the resulting plates could be considered high quality castings. It is expected that much better results would have been obtained if the die temperature had been increased to approximately 300°C and the slugs were heated in the multi-stage induction heater.

As illustrated by the tests, if the gate speed is too high, the metal flow will not be laminar. Too low a gate speed results in metal solidification before the mold cavity fills.

Despite the less than optimal casting conditions, as illustrated by example 3 below, the cast plates show good physical properties.

The casting machine was a single cylinder unit having servo control to carefully control the force driving the slug into the closed die. Optimally the casting process will cause the outer skin of the slug which contains surface oxides resulting from the heating process to be removed from the virgin metal.

### EXAMPLE 3

Plates 34 and 35 were sectioned into six sections as illustrated in Figure 30. One quarter inch (1/4 in.) round samples were removed from the sections and tested for mechanical properties. The plates were not heat treated and the results are tabulated in Table 1 below.

**TABLE 1**

| PLATE NO. | SAMPLE NO. | SAMPLE TYPE | UTS (ksi) | YS (ksi) | ELONG % |
|---|---|---|---|---|---|
| 34 | 2 | .250" ROUND | 31.5 | 13.9 | 10.9 |
| 34 | 4 | .250" ROUND | 33.2 | 14.2 | 14.1 |
| 34 | 6 | .250" ROUND | 32.9 | 14.5 | 13.6 |
| 35 | 2 | .250" ROUND | 33.6 | 14.7 | 12.3 |
| 35 | 4 | .250" ROUND | 31.1 | 13.9 | 10.3 |
| 35 | 6 | .250" ROUND | 33.3 | 13.9 | 13.3 |

Plates 34 and 35 were subsequently solution heat treated for 12 hours at 426°C and still air cooled. One quarter inch (1/4 in.) round samples were cut from the plates and the mechanical properties of those samples were tested. The results of the tests are tabulated in Table 2 below. In Table 2 below the sample plan for the heat treated plates is the same as illustrated in Figure 31.

**TABLE 2**

| PLATE NO. | SAMPLE NO. | SAMPLE TYPE | UTS (ksi) | YS (ksi) | ELONG % | COMMENTS |
|---|---|---|---|---|---|---|
| 34 | 1 | .250" ROUND | 23.4 | 14.1 | 3.0 | OXIDE INCL. |
| 34 | 3 | .250" ROUND | SAMPLE DAMAGED IN MACHINING | | | |
| 34 | 5 | .250" ROUND | 37.6 | 14.6 | 18.5 | |
| 35 | 1 | .250" ROUND | 37.0 | 12.8 | 15.7 | |
| 35 | 3 | .250" ROUND | 36.9 | 13.8 | 16.4 | |
| 35 | 5 | .250" ROUND | 36.8 | 12.8 | 19.3 | |

Photomicrographs of one of the plates were taken at locations M1 and M2 as illustrated in Figure 32. The photomicrographs are reproduced in Figures 33 through 36 as follows:
Figure 33 is a photomicrograph of sample M1 at 50x magnification;
Figure 34 is a photomicrograph of sample M1 at 100x magnification;
Figure 35 is a photomicrograph of sample M2 at 50x magnification;
Figure 36 is a photomicrograph of sample M2 at 100x magnification.

The above description is intended in an illustrative rather than a restrictive sense. One skilled in the art would recognize that the specific process perameters used in the examples would have to be varied to adapt the present invention to particular alloys, equipment and parts being cast. For example, although AZ61 magesium alloy was utilized in the tests no doubt other magesium alloys could be used. The process can also be adapted to metal systems other than magesium where the metal is capable of forming a two-phase system comprising **a solid particles** in a lower melting matrix. The process will work with aluminum and may also work with other similar metal systems such as copper.

Preferably heating of the billet 22 prior to forming should be carried out at a rate of no greater than 30°C per second and even more preferably at a rate of no greater than 20°C per second if aluminum is being used. Heating at a rate greater than 30°C per second may result in the precipitation of silicon from the resulting stresses thereby deleteriously affecting machinability of the finished part. It has been found that a three stage induction heater is particularly well suited to maintaining a desirable heating rate.

## Claims

1. A process for producing a billet for use in a semi-solid metal forming process having the following steps:
i) obtaining a direct chill cast billet which was cooled at a rate exceeding 2°C per second during its production;
ii) heating the direct chill cast billet of step i) to a temperature above its recrystallization temperature and below its solidus temperature;
iii) reducing the diameter of the heated billet from step ii) and breaking down its grain structure by extruding it through an extruding die to form an extruded column; and,
iv) cutting the extruded column to form said billet.

2. A process as claimed in claim 1 wherein the direct chill cast billet used in step
i) has a maximum grain size of less than 100 microns.

3. A billet for use in a semi-solid metal forming process, the billet being obtainable by a process according to any preceding claim.

4. A semi-solid metal forming process having the following steps:
i) obtaining a direct chill cast billet which, during its production, was cooled at a rate exceeding 2°C per second;
ii) heating the direct chill cast billet to a temperature above its recrystallization temperature and below its solidus temperature;
iii) reducing the diameter of the heated billet from step i) and breaking down its grain structure by extruding it through an extruding die to form an extruded column;
iv) cutting the extruded column into billets;
v) heating the billet from step iv) to a forming temperature above its solidus and below its liquidus temperature;
vi) forming a part from the heated billet by (a) placing the heated billet into an injection chamber in a semi-solid die casting machine, injecting the heated billet section into a mold to form a part; and removing the part from the mold; or (b) placing the heated billet between a set of dies in a forging machine, actuating the forging machine to squeeze the billet between the set of dies to form a part, and separating the dies and removing the part.

5. A semi-solid metal forming process as claimed in claim 4 wherein the direct chill cast billet used in step i) has a maximum grain size of less than 100 microns.

6. A semi-solid metal forming process as claimed in claim 5 wherein a suitable alloy of aluminum is used and is heated in step v) in a three stage induction heater at a rate not exceeding 30°C per second.

7. A semi-solid metal forming process as claimed in claim 6 wherein the heating rate in step v) does not exceed 20°C per second.

8. A semi-solid metal forming process as claimed in claim 6 wherein in step v) the billet is heated to its forming temperature at a rate between 20°C per second and 30°C per second.

9. A semi-solid metal forming process as claimed in claim 4 wherein:
- the direct chill cast billet is of AZ61 magnesium alloy which, during its production, was cooled at a rate exceeding 2°C per second;
- at step (ii) the billet is heated to a temperature of approximately 300°C, and;
- at step (iii) the billet is extruded into an extruded column at a temperature of from about 330 to 350°C.

## Patentansprüche

1. Verfahren zum Herstellen eines Blocks zur Verwendung in einem Halbfest-Metallumformverfahren mit den folgenden Schritten:
i) Beschaffen eines Kokillengussblocks im Bruttozustand, der während seiner Herstellung mit einer Rate von über 2°C pro Sekunde gekühlt wurde;
ii) Erwärmen des Kokillengussblocks im Bruttozustand von Schritt i) auf eine Temperatur über seiner Rekristallisationstemperatur und unter seiner Festzustandstemperatur;
iii) Verringern des Durchmessers des erwärmten Blocks von Schritt ii) und Abbauen seiner Kornstruktur, indem er durch ein Strangpresswerkzeug gepresst wird zum Formen einer stranggepressten Säule und
iv) Schneiden der stranggepressten Säule zum Formen des genannten Blocks.

2. Verfahren nach Anspruch 1, bei dem der in Schritt i) verwendete Kokillengussblock im Bruttozustand eine maximale Korngröße von weniger als 100 Mikrometern hat.

3. Block zur Verwendung in einem Halbfest-Metallumformverfahren, wobei der Block durch ein Verfahren nach einem der vorhergehenden Ansprüche erhaltbar ist.

4. Halbfest-Metallumformverfahren mit den folgenden Schritten:
i) Beschaffen eines Kokillengussblocks im Bruttozustand, der während seiner Herstellung mit einer Rate von über 2°C pro Sekunde gekühlt wurde;
ii) Erwärmen des Kokillengussblocks im Bruttozustand auf eine Temperatur über seiner Rekristallisationstemperatur und unter seiner Festzustandstemperatur;
iii) Verringern des Durchmessers des erwärmten Blocks von Schritt i) und Zersetzen seiner Kornstruktur, indem er durch ein Strangpresswerkzeug gepresst wird zum Formen einer stranggepressten Säule;
iv) Schneiden der stranggepressten Säule in Blöcke;
v) Erwärmen des Blocks von Schritt iv) auf eine Umformtemperatur über seinem festen Zustand und unter seiner Flüssigzustandtemperatur;
vi) Formen eines Teils aus dem erwärmten Block, indem (a) der erwärmte Block in eine Einspritzkammer in einer Halbfestdruckgussmaschine gegeben wird, der erwärmte Blockabschnitt in eine Form gespritzt wird, um ein Teil zu formen, und das Teil aus der Form entfernt wird; oder b) der erwärmte Block zwischen einen Werkzeugsatz in einer Schmiedemaschine gegeben wird, die Schmiedemaschine betätigt wird, um den Block zum Formen eines Teils zwischen den Werkzeugsätzen zu quetschen, und die Werkzeuge getrennt werden und das Teil entfernt wird.

5. Halbfest-Metallumformverfahren nach Anspruch 4, bei dem der in Schritt i) verwendete Kokillengussblock im Bruttozustand eine maximale Korngröße von weniger als 100 Mikrometern hat.

6. Halbfest-Metallumformverfahren nach Anspruch 5, bei dem eine geeignete Aluminiumlegierung verwendet wird und in Schritt v) in einem Dreistufen-Induktionsheizgerät mit einer Rate von höchstens 30° pro Sekunde erwärmt wird.

7. Halbfest-Metallumformverfahren nach Anspruch 6, bei dem die Erwärmungsrate in Schritt v) 20°C pro Sekunde nicht überschreitet.

8. Halbfest-Metallumformverfahren nach Anspruch 6, bei dem der Block in Schritt v) mit einer Rate zwischen 20°C pro Sekunde und 30°C pro Sekunde auf seine Umformtemperatur erwärmt wird.

9. Halbfest-Metallumformverfahren nach Anspruch 4, bei dem:
- der Kokillengussblock im Bruttozustand aus AZ61-Magnesiumlegierung ist, die während ihrer Herstellung mit einer Rate über 2°C pro Sekunde gekühlt wurde;
- der Block an Schritt (ii) auf eine Temperatur von ungefähr 300°C erwärmt wird und
- der Block an Schritt (iii) bei einer Temperatur von ungefähr 330 bis 350°C zu einer gepressten Säule stranggepresst wird.

## Revendications

1. Processus pour produire une billette à utiliser dans un processus de formage de métal semi-solide comprenant les étapes suivantes :
i) obtention d'une billette coulée en coquille en première fusion qui a été refroidie à une cadence dépassant 2 °C par seconde pendant sa production ;
ii) chauffage de la billette coulée en coquille en première fusion de l'étape i) à une température supérieure à sa température de recristallisation et inférieure à sa température de solidus ;
iii) réduction du diamètre de la billette chauffée de l'étape ii) et décomposition de sa structure granulaire en l'extrudant à travers une filière d'extrusion pour former une colonne extrudée, et
iv) découpage de la colonne extrudée pour former ladite billette.

2. Processus suivant la revendication 1, dans lequel la billette coulée en coquille en première fusion utilisée à l'étape i) présente une taille de grain maximum inférieure à 100 microns.

3. Billette à utiliser dans un processus de formage de métal semi-solide, la billette pouvant être obtenue par un processus suivant l'une quelconque des revendications précédentes.

4. Processus de formage de métal semi-solide comprenant les étapes suivantes :
i) obtention d'une billette coulée en coquille en première fusion qui, pendant sa production, a été refroidie à une cadence dépassant 2 °C par seconde ;
ii) chauffage de la billette coulée en coquille en première fusion à une température supérieure à sa température de recristallisation et inférieure à sa température de solidus ;
iii) réduction du diamètre de la billette chauffée de l'étape i) et décomposition de sa structure granulaire en l'extrudant à travers une filière d'extrusion pour former une colonne extrudée ;
iv) découpage de la colonne extrudée en billettes ;
v) chauffage de la billette de l'étape iv) à une température de formage supérieure à sa température de solidus et inférieure à sa température de liquidus, et
vi) formage d'une pièce à partir de la billette chauffée (a) en plaçant la billette chauffée dans une chambre d'injection dans une machine à couler sous pression semi-solide, en injectant la section de billette chauffée dans un moule pour former une pièce, et en retirant la pièce du moule ; ou (b) en plaçant la billette chauffée entre un jeu de filières dans une machine à forger, en actionnant la machine à forger pour presser la billette entre le jeu de filières pour former une pièce et en séparant les filières et en retirant la pièce.

5. Processus de formage de métal semi-solide suivant la revendication 4, dans lequel la billette coulée en coquille en première fusion utilisée à l'étape i) présente une taille granulaire maximum inférieure à 100 microns.

6. Processus de formage de métal semi-solide suivant la revendication 5, dans lequel un alliage approprié d'aluminium est utilisé et est chauffé à l'étape v) dans un four à induction à trois étages à une cadence ne dépassant pas 30 °C par seconde.

7. Processus de formage de métal semi-solide suivant la revendication 6, dans lequel la cadence de chauffage à l'étape v) ne dépasse pas 20 °C par seconde.

8. Processus de formage de métal semi-solide suivant la revendication 6, dans lequel à l'étape v) la billette est chauffée à sa température de formage à une cadence comprise entre 20 °C par seconde et 30 °C par seconde.

9. Processus de formage de métal semi-solide suivant la revendication 4, dans lequel :
- la billette coulée en coquille en première fusion est d'un alliage de magnésium AZ61 qui, pendant sa production, a été refroidi à une cadence dépassant 2 °C par seconde ;
- à l'étape (ii) la billette est chauffée à une température d'environ 300 °C, et
- à l'étape (iii) la billette est extrudée en une colonne extrudée à une température comprise entre environ 330 et 350 °C.
